



US007807099B2

(12) **United States Patent**  
**Choe et al.**

(10) **Patent No.:** **US 7,807,099 B2**  
(45) **Date of Patent:** **Oct. 5, 2010**

(54) **METHOD FOR FORMING EARTH-BORING  
TOOLS COMPRISING SILICON CARBIDE  
COMPOSITE MATERIALS**

(75) Inventors: **Heeman Choe**, Seoul (KR); **John H. Stevens**, Spring, TX (US); **James C. Westhoff**, The Woodlands, TX (US); **Jimmy W. Eason**, The Woodlands, TX (US); **James L. Overstreet**, Tomball, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 0 days.

(21) Appl. No.: **11/965,018**

(22) Filed: **Dec. 27, 2007**

(65) **Prior Publication Data**

US 2008/0128176 A1 Jun. 5, 2008

**Related U.S. Application Data**

(63) Continuation-in-part of application No. 11/271,153, filed on Nov. 10, 2005, and a continuation-in-part of application No. 11/272,439, filed on Nov. 10, 2005.

(51) **Int. Cl.**  
**B22F 3/12** (2006.01)

(52) **U.S. Cl.** ..... **419/14**; 419/31; 419/33;  
419/55

(58) **Field of Classification Search** ..... 419/8,  
419/14, 31, 33, 55

See application file for complete search history.

(56) **References Cited**

**U.S. PATENT DOCUMENTS**

- 1,676,887 A 7/1928 Chamberlin  
2,299,207 A \* 10/1942 Bevillard ..... 76/108.1  
3,757,878 A 9/1973 Wilder et al.  
3,757,879 A 9/1973 Wilder et al.  
3,841,852 A 10/1974 Wilder et al.  
4,098,363 A 7/1978 Rohde et al.  
4,134,759 A \* 1/1979 Yajima et al. ..... 419/17  
4,981,665 A \* 1/1991 Boecker et al. ..... 423/345  
6,284,014 B1 \* 9/2001 Carden ..... 75/252  
6,503,572 B1 1/2003 Aghajanian et al.  
6,862,970 B2 3/2005 Waggoner et al.  
6,919,127 B2 7/2005 Waggoner et al.  
6,995,103 B2 2/2006 Aghajanian  
2005/0247491 A1 \* 11/2005 Mirchandani et al. ..... 175/374  
2007/0102198 A1 5/2007 Oxford et al.  
2007/0102199 A1 5/2007 Smith et al.  
2007/0102200 A1 5/2007 Choe et al.  
2007/0102202 A1 5/2007 Choe et al.

**OTHER PUBLICATIONS**

Al-Haidary, J.T., et al., "Evaluation Study of Cast Al-SiCp composites," Materials Science-Poland, vol. 25, No. 1, 2007.

Basavarajappa, S., et al., "Dry Sliding Wear Behaviour of Al 2219/SiC Metal Matrix Composites," Materials Science-Poland, vol. 24, No. 2/1, 2006.

Chen, D., et al., "Mechanisms of High-Temperature Fatigue in Silicon Carbide Ceramics," Fatigue and Fracture Behavior of High Temperature Materials, TMS (The Minerals, Metals & Materials Society), Warrendale, PA, pp. 1-8, 2000.

Chen, D., et al., "High-Temperature Cyclic Fatigue-Crack Growth Behavior in an In Situ Toughened Silicon Carbide," Acta mater., vol. 48, pp. 659-674, 2000.

Chen, D., et al., "Role of the Grain-Boundary Phase on the Elevated-Temperature Strength, Toughness, Fatigue and Creep Resistance of Silicon Carbide Sintered with Al, B and C," Acta mater., vol. 48, pp. 4599-4608, 2000.

Key-To-Nonferrous, "Aluminum Matrix Composites with Discontinuous Silicon Carbide Reinforcement," <http://www.key-to-nonferrous.com>, 3 pages, downloaded Aug. 27, 2007.

Mabuchi, M., et al., "Very High Strain-Rate Superplasticity in a Particulate Si3N4/6061 Aluminum Composite," Scripta Metallurgica et Materialia, vol. 25, No. 11, pp. 2517-2520, Copyright (c) 1991 Pergamon Press plc.

M Cubed Technologies Inc., "Cast Silicon Carbide Particulate-Reinforced Aluminum (Al/SiC) Metal Matrix Composites," Technote, Cast MMC, Rev. 02, 3 pages, May 8, 2001.

Moberlychan, W.J., et al., "Controlling Interface Chemistry and Structure to Process and Toughen Silicon Carbide," Acta mater., vol. 46, No. 7, pp. 2471-2477, 1998.

Moberlychan, W.J., et al., "The Roles of Amorphous Grain Boundaries and the  $\beta$ - $\alpha$  Transformation in Toughening SiC," Acta mater., vol. 46, No. 5, pp. 1625-1635, 1998.

Pruthviraj, R.D., et al., "Friction and Wear of Al6061 Containing 10wt.% Sic Metal Matrix Composites," International Journal of Material Science, vol. 2, No. 1, pp. 59-64, 2007.

Yang, Guang, et al., "Chemical Reaction in Al Matrix Composite Reinforced with Sicp Coated by SnO<sub>2</sub>," Journal of Materials Science, vol. 39, pp. 3689-3694, 2004.

Yuan, R., et al., "Ambient to High-Temperature Fracture Toughness and Cyclic Fatigue Behavior in Al-Containing Silicon Carbide Ceramics," Acta mater., vol. 51, pp. 6477-6491, 2003.

Zhang, Xiao Feng, et al., "Abrasive Wear Behavior of Heat-Treated ABC-Silicon Carbide," J. Am. Ceram. Soc., vol. 86, No. 8, pp. 1370-1378, 2003.

PCT International Search Report for International Application No. PCT/US2008/087647, mailed Jul. 23, 2009.

\* cited by examiner

*Primary Examiner*—Roy King

*Assistant Examiner*—Ngoclan T Mai

(74) *Attorney, Agent, or Firm*—TraskBritt

(57) **ABSTRACT**

Earth-boring tools for drilling subterranean formations include a particle-matrix composite material comprising a plurality of silicon carbide particles dispersed throughout a matrix material, such as, for example, an aluminum or aluminum-based alloy. In some embodiments, the silicon carbide particles comprise an ABC—SiC material. Methods of manufacturing such tools include providing a plurality of silicon carbide particles within a matrix material. Optionally, the silicon carbide particles may comprise ABC—SiC material, and the ABC—SiC material may be toughened to increase a fracture toughness exhibited by the ABC—SiC material. In some methods, at least one of an infiltration process and a powder compaction and consolidation process may be employed.



FIG. 1



FIG. 2



FIG. 3

**FIG. 4**

**METHOD FOR FORMING EARTH-BORING  
TOOLS COMPRISING SILICON CARBIDE  
COMPOSITE MATERIALS**

**CROSS-REFERENCE TO RELATED  
APPLICATIONS**

This application is a continuation-in-part of each of pending application Ser. No. 11/271,153, filed Nov. 10, 2005, and pending application Ser. No. 11/272,439, filed Nov. 10, 2005, the disclosure of each of which application is incorporated herein in its entirety by this reference.

**TECHNICAL FIELD**

The present invention generally relates to earth-boring tools, and to methods of manufacturing such earth-boring tools. More particularly, the present invention generally relates to earth-boring tools that include a body having at least a portion thereof substantially formed of a particle-matrix composite material, and to methods of manufacturing such earth-boring tools.

**BACKGROUND**

Rotary drill bits are commonly used for drilling bore holes, or well bores, in earth formations. Rotary drill bits include two primary configurations. One configuration is the roller cone bit, which conventionally includes three roller cones mounted on support legs that extend from a bit body. Each roller cone is configured to spin or rotate on a support leg. Teeth are provided on the outer surfaces of each roller cone for cutting rock and other earth formations. The teeth often are coated with an abrasive, hard ("hardfacing") material. Such materials often include tungsten carbide particles dispersed throughout a metal alloy matrix material. Alternatively, receptacles are provided on the outer surfaces of each roller cone into which hard metal inserts are secured to form the cutting elements. In some instances, these inserts comprise a superabrasive material formed on and bonded to a metallic substrate. The roller cone drill bit may be placed in a bore hole such that the roller cones abut against the earth formation to be drilled. As the drill bit is rotated under applied weight on bit, the roller cones roll across the surface of the formation, and the teeth crush the underlying formation.

A second primary configuration of a rotary drill bit is the fixed-cutter bit (often referred to as a "drag" bit), which conventionally includes a plurality of cutting elements secured to a face region of a bit body. Generally, the cutting elements of a fixed-cutter type drill bit have either a disk shape or a substantially cylindrical shape. A hard, superabrasive material, such as mutually bonded particles of polycrystalline diamond, may be provided on a substantially circular end surface of each cutting element to provide a cutting surface. Such cutting elements are often referred to as "polycrystalline diamond compact" (PDC) cutters. The cutting elements may be fabricated separately from the bit body and are secured within pockets formed in the outer surface of the bit body. A bonding material such as an adhesive or a braze alloy may be used to secure the cutting elements to the bit body. The fixed-cutter drill bit may be placed in a bore hole such that the cutting elements abut against the earth formation to be drilled. As the drill bit is rotated, the cutting elements scrape across and shear away the surface of the underlying formation.

The bit body of a rotary drill bit of either primary configuration may be secured, as is conventional, to a hardened steel

shank having an American Petroleum Institute (API) threaded pin for attaching the drill bit to a drill string. The drill string includes tubular pipe and equipment segments coupled end-to-end between the drill bit and other drilling equipment at the surface. Equipment such as a rotary table or top drive may be used for rotating the drill string and the drill bit within the bore hole. Alternatively the shank of the drill bit may be coupled directly to the drive shaft of a down-hole motor, which then may be used to rotate the drill bit.

10 The bit body of a rotary drill bit may be formed from steel. Alternatively, the bit body may be formed from a particle-matrix composite material. Such particle-matrix composite materials conventionally include hard tungsten carbide particles randomly dispersed throughout a copper or copper-based alloy matrix material (often referred to as a "binder" material). Such bit bodies conventionally are formed by embedding a steel blank in tungsten carbide particulate material within a mold, and infiltrating the particulate tungsten carbide material with molten copper or copper-based alloy material. Drill bits that have bit bodies formed from such particle-matrix composite materials may exhibit increased erosion and wear resistance, but lower strength and toughness, relative to drill bits having steel bit bodies.

15 As subterranean drilling conditions and requirements become ever more rigorous, there arises a need in the art for novel particle-matrix composite materials for use in bit bodies of rotary drill bits that exhibit enhanced physical properties and that may be used to improve the performance of earth-boring rotary drill bits.

**BRIEF SUMMARY OF THE INVENTION**

20 In some embodiments, the present invention includes earth-boring tools for drilling subterranean formations. The tools include a bit body comprising a composite material. The composite material includes a first discontinuous phase within a continuous matrix phase. The first discontinuous phase includes silicon carbide. In some embodiments, the discontinuous phase may comprise silicon carbide particles, and the continuous matrix phase may comprise aluminum or an aluminum-based alloy. Furthermore, the first discontinuous phase may optionally comprise what may be referred to as an ABC—SiC material, as discussed in further detail below. Optionally, such ABC—SiC materials may comprise toughened ABC—SiC materials that exhibit increased fracture toughness relative to conventional silicon carbide materials.

25 In further embodiments, the present invention includes methods of forming earth-boring tools. The methods include providing a plurality of silicon carbide particles in a matrix material to form a body, and shaping the body to form at least a portion of an earth-boring tool for drilling subterranean formations. In some embodiments, the silicon carbide particles may comprise an ABC—SiC material. Optionally, such ABC—SiC materials may be toughened to cause the ABC—SiC materials to exhibit increased fracture toughness relative to conventional silicon carbide materials. In some embodiments, silicon carbide particles may be infiltrated with a molten matrix material, such as, for example, an aluminum or aluminum-based alloy. In additional embodiments, a green powder component may be provided that includes a plurality of particles comprising silicon carbide and a plurality of particles comprising matrix material, and the green powder component may be at least partially sintered.

30 In still further embodiments, the present invention includes methods of forming at least a portion of an earth-boring tool. An ABC—SiC material may be consolidated to form one or more compacts, and the compacts may be broken apart to

form a plurality of ABC—SiC particles. At least a portion of a body of an earth-boring tool may be formed to comprise a composite material that includes the plurality of ABC—SiC particles. Optionally, such ABC—SiC materials may be toughened to cause the ABC—SiC materials to exhibit increased fracture toughness relative to conventional silicon carbide materials.

#### BRIEF DESCRIPTION OF THE SEVERAL VIEWS OF THE DRAWINGS

While the specification concludes with claims particularly pointing out and distinctly claiming that which is regarded as the present invention, the advantages of this invention may be more readily ascertained from the following description of the invention when read in conjunction with the accompanying drawings in which:

FIG. 1 is a partial cross-sectional side view of an earth-boring rotary drill bit that embodies teachings of the present invention and includes a bit body comprising a particle-matrix composite material;

FIG. 2 is an illustration representing one example of how a microstructure of the particle-matrix composite material of the bit body of the drill bit shown in FIG. 1 may appear in a micrograph at a first level of magnification;

FIG. 3 is an illustration representing one example of how the microstructure of the particles of the particle-matrix composite material shown in FIG. 2 may appear at a relatively higher level of magnification; and

FIG. 4 is an illustration representing one example of how the microstructure of the matrix material of the particle-matrix composite material shown in FIG. 2 may appear at a relatively higher level of magnification.

#### DETAILED DESCRIPTION OF THE INVENTION

The illustrations presented herein are not meant to be actual views of any particular material, apparatus, or method, but are merely idealized representations which are employed to describe embodiments of the present invention. Additionally, elements common between figures may retain the same numerical designation.

An embodiment of an earth-boring rotary drill bit 10 of the present invention is shown in FIG. 1. The drill bit 10 includes a bit body 12 comprising a particle-matrix composite material 15 that includes a plurality of silicon carbide particles dispersed throughout an aluminum or an aluminum-based alloy matrix material. By way of example and not limitation, the bit body 12 may include a crown region 14 and a metal blank 16. The crown region 14 may be predominantly comprised of the particle-matrix composite material 15, as shown in FIG. 1. The metal blank 16 may comprise a metal or metal alloy, and may be configured for securing the crown region 14 of the bit body 12 to a metal shank 20 that is configured for securing the drill bit 10 to a drill string (not shown). The metal blank 16 may be secured to the crown region 14 during fabrication of the crown region 14, as discussed in further detail below. In additional embodiments, however, the drill bit 10 may not include a metal blank 16.

FIG. 2 is an illustration providing one example of how the microstructure of the particle-matrix composite material 15 may appear in a magnified micrograph acquired using, for example, an optical microscope, a scanning electron microscope (SEM), or other instrument capable of acquiring or generating a magnified image of the particle-matrix composite material 15. As shown in FIG. 2, the particle-matrix composite material 15 may include a plurality of silicon carbide

(SiC) particles dispersed throughout an aluminum or an aluminum-based alloy matrix material 52. In other words, the particle-matrix composite material 15 may include a plurality of discontinuous silicon carbide (SiC) phase regions dispersed throughout a continuous aluminum or an aluminum-based alloy phase. By way of example and not limitation, in some embodiments, the silicon carbide particles 50 may comprise between about forty percent (40%) and about seventy percent (70%) by weight of the particle-matrix composite material 15, and the matrix material 52 may comprise between about thirty percent (30%) and about sixty percent (60%) by weight of the particle-matrix composite material 15. In additional embodiments, the silicon carbide particles 50 may comprise between about seventy percent (70%) and about ninety-five percent (95%) by weight of the particle-matrix composite material 15, and the matrix material 52 may comprise between about thirty percent (30%) and about five percent (5%) by weight of the particle-matrix composite material 15.

As shown in FIG. 2, in some embodiments, the silicon carbide particles 50 may have different sizes. For example, the plurality of silicon carbide particles 50 may include a multi-modal particle size distribution (e.g., bi-modal, tri-modal, tetra-modal, penta-modal, etc.). In other embodiments, however, the silicon carbide particles 50 may have a substantially uniform particle size, which may exhibit a Gaussian or log-normal distribution. By way of example and not limitation, the plurality of silicon carbide particles 50 may include a plurality of -70 ASTM (American Society for Testing and Materials) mesh silicon carbide particles. As used herein, the phrase “-70 ASTM mesh particles” means particles that pass through an ASTM No. 70 U.S.A. standard testing sieve as defined in ASTM Specification E11-04, which is entitled Standard Specification for Wire Cloth and Sieves for Testing Purposes.

The silicon carbide particles 50 may comprise, for example, generally rough, non-rounded (e.g., polyhedron-shaped) particles or generally smooth, rounded particles. In some embodiments, each silicon carbide particle 50 may comprise a plurality of individual silicon carbide grains, which may be bonded to one another. Such interbonded silicon carbide grains in the silicon carbide particles 50 may be generally plate-like, or they may be generally elongated. For example, the interbonded silicon carbide gains may have an aspect ratio (the ratio of the average particle length to the average particle width) of greater than about five (5) (e.g., between about five (5) and about nine (9)).

FIG. 3 illustrates one example of how the microstructure of the silicon carbide particles 50 shown in FIG. 2 may appear at a relatively higher level of magnification. As shown in FIG. 3, each silicon carbide particle 50 may, in some embodiments, comprise a plurality of interlocked elongated and/or plate-shaped grains 51 comprising silicon carbide (and, optionally, an ABC—SiC material, which may comprise an in situ toughened ABC—SiC material).

In some embodiments, the silicon carbide particles 50 may comprise small amounts of aluminum (Al), boron (B), and carbon (C). For example, the silicon carbide material in the silicon carbide particles 50 may comprise between about one percent by weight (1.0 wt %) and about five percent by weight (5.0 wt %) aluminum, less than about one percent by weight (1.0 wt %) boron, and between about one percent by weight (1.0 wt %) and about four percent by weight (4.0 wt %) carbon. Such silicon carbide materials are referred to in the art as “ABC—SiC” materials, and may exhibit physical properties that are relatively more desirable than conventional SiC materials for purposes of forming the particle-matrix com-

posite material **15** of the bit body **12** of the earth-boring rotary drill bit **10**. As one non-limiting example, the silicon carbide material in the silicon carbide particles **50** may comprise about three percent by weight (3.0 wt %) Aluminum, about

silicon carbide particles **50**. Table 1 below sets forth various examples of compositions of matrix material **52** that may be used as the particle-matrix composite material **15** of the crown region **14** of the bit body **12** shown in FIG. 1.

TABLE 1

| Example No. | Approximate Elemental Weight Percent |      |      |      |      |      |      |     |      |      |      |      |
|-------------|--------------------------------------|------|------|------|------|------|------|-----|------|------|------|------|
|             | Al                                   | Cu   | Mg   | Mn   | Si   | Zr   | Fe   | Cr  | Ni   | Sn   | Ti   | Zn   |
| 1           | 95.0                                 | 5.0  | —    | —    | —    | —    | —    | —   | —    | —    | —    | —    |
| 2           | 96.5                                 | 3.5  | —    | —    | —    | —    | —    | —   | —    | —    | —    | —    |
| 3           | 94.5                                 | 4.0  | 1.5  | —    | —    | —    | —    | —   | —    | —    | —    | —    |
| 4           | 93.5                                 | 4.4  | 0.5  | 0.8  | 0.8  | —    | —    | —   | —    | —    | —    | —    |
| 5           | 93.4                                 | 4.5  | 1.5  | 0.6  | —    | —    | —    | —   | —    | —    | —    | —    |
| 6           | 93.5                                 | 4.4  | 1.5  | 0.6  | —    | —    | —    | —   | —    | —    | —    | —    |
| 7           | 89.1                                 | 2.3  | 2.3  | —    | 0.1  | —    | —    | —   | —    | —    | 6.2  | —    |
| 8           | 50.0                                 | —    | —    | —    | 50.0 | —    | —    | —   | —    | —    | —    | —    |
| 9           | 99.0                                 | 0.10 | —    | —    | 0.15 | —    | 0.7  | —   | —    | —    | —    | 0.05 |
| 10          | 92.2                                 | 4.5  | 0.30 | 2.5  | 0.10 | —    | 0.15 | —   | —    | —    | 0.25 | —    |
| 11          | 87.3                                 | 3.5  | 0.1  | 0.5  | 6.0  | —    | 1.0  | —   | 0.35 | —    | 0.25 | 1.0  |
| 12          | 83.4                                 | 1.0  | 0.1  | 0.35 | 12.0 | —    | 2.0  | —   | 0.5  | 0.15 | —    | 0.5  |
| 13          | 94.0                                 | 0.15 | 4.25 | 0.35 | 0.35 | 0.15 | 0.5  | —   | —    | —    | 0.25 | —    |
| 14          | 93.5                                 | 0.2  | 1.4  | 0.4  | 0.2  | —    | 0.8  | 0.3 | —    | —    | 0.25 | 2.95 |
| 15          | 90.2                                 | 1.0  | 0.1  | 0.1  | 0.7  | —    | 0.7  | —   | 1.0  | 6.0  | 0.2  | —    |

six tenths of one percent by weight (0.6 wt %) boron, and about two percent by weight (2.0 wt %) carbon. In some embodiments, the silicon carbide particles **50** may comprise an ABC—SiC material that exhibits a fracture toughness of about five megapascal root meters (5.0 MPa-m<sup>1/2</sup>) or more. More particularly, the silicon carbide particles **50** may comprise an ABC—SiC material that exhibits a fracture toughness of about six megapascal root meters (6.0 MPa-m<sup>1/2</sup>) or more. In yet further embodiments, the silicon carbide particles **50** may comprise an ABC—SiC material that exhibits a fracture toughness of about nine megapascal root meters (9.0 MPa-m<sup>1/2</sup>) or more. Optionally, the silicon carbide particles **50** may comprise an in situ toughened ABC—SiC material, as discussed in further detail below. Such in situ toughened ABC—SiC materials may exhibit a fracture toughness greater than about five megapascal root meters (5 MPa-m<sup>1/2</sup>), or even greater than about six megapascal root meters (6 MPa-m<sup>1/2</sup>). In some embodiments, the in situ toughened ABC—SiC materials may exhibit a fracture toughness greater than about nine megapascal root meters (9 MPa-m<sup>1/2</sup>).

In some embodiments, the silicon carbide particles **50** may comprise a coating comprising a material configured to enhance the wettability of the silicon carbide particles **50** to the matrix material **52** and/or to prevent any detrimental chemical reaction from occurring between the silicon carbide particles **50** and the surrounding matrix material **52**. By way of example and not limitation, the silicon carbide particles **50** may comprise a coating of at least one of tin oxide (SnO<sub>2</sub>), tungsten, nickel, and titanium.

In some embodiments of the present invention, the bulk matrix material **52** may include at least seventy-five percent by weight (75 wt %) aluminum, and at least trace amounts of at least one of boron, carbon, copper, iron, lithium, magnesium, manganese, nickel, scandium, silicon, tin, zirconium, and zinc. Furthermore, in some embodiments, the matrix material **52** may include at least ninety percent by weight (90 wt %) aluminum, and at least three percent by weight (3 wt %) of at least one of boron, carbon, copper, magnesium, manganese, scandium, silicon, zirconium, and zinc. Furthermore, trace amounts of at least one of silver, gold, and indium optionally may be included in the matrix material **52** to enhance the wettability of the matrix material relative to the

FIG. 4 is an enlarged view of a region of the matrix material **52** shown in FIG. 2. FIG. 4 illustrates one example of how the microstructure of the matrix material **52** of the particle-matrix composite material **15** may appear in a micrograph at an even greater magnification level than that represented in FIG. 2. Such a micrograph may be acquired using, for example, a scanning electron microscope (SEM) or a transmission electron microscope (TEM).

By way of example and not limitation, the matrix material **52** may include a continuous phase **54** comprising a solid solution. The matrix material **52** may further include a discontinuous phase **56** comprising a plurality of discrete regions, each of which includes precipitates (i.e., a precipitate phase). In other words, the matrix material **52** may comprise a precipitation hardened aluminum-based alloy comprising between about ninety-five percent by weight (95 wt %) and about ninety-six and one-half percent by weight (96.5 wt %) aluminum and between about three and one-half percent by weight (3.5 wt %) and about five percent by weight (5 wt %) copper. In such a matrix material **52**, the solid solution of the continuous phase **54** may include aluminum solvent and copper solute. In other words, the crystal structure of the solid solution may comprise mostly aluminum atoms with a relatively small number of copper atoms substituted for aluminum atoms at random locations throughout the crystal structure. Furthermore, in such a matrix material **52**, the discontinuous phase **56** of the matrix material **52** may include one or more intermetallic compound precipitates (e.g., CuAl<sub>2</sub>). In additional embodiments, the discontinuous phase **56** of the matrix material **52** may include additional discontinuous phases (not shown) present in the matrix material **52** that include metastable transition phases (i.e., non-equilibrium phases that are temporarily formed during formation of an equilibrium precipitate phase (e.g., CuAl<sub>2</sub>)). Furthermore, in yet additional embodiments, substantially all of the discontinuous phase **56** regions may be substantially comprised of such metastable transition phases. The presence of the discontinuous phase **56** regions within the continuous phase **54** may impart one or more desirable properties to the matrix material **52**, such as, for example, increased hardness. Furthermore, in some embodiments, metastable transition phases may impart one or more physical properties to the

matrix material 52 that are more desirable than those imparted to the matrix material 52 by equilibrium precipitate phases (e.g., CuAl<sub>2</sub>).

With continued reference to FIG. 4, the matrix material 52 may include a plurality of grains 60 that abut one another along grain boundaries 62. As shown in FIG. 4, a relatively high concentration of a discontinuous precipitate phase 56 may be present along the grain boundaries 62. In some embodiments of the present invention, the grains 60 of matrix material 52 may have at least one of a size and shape that is tailored to enhance one or more mechanical properties of the matrix material 52. For example, in some embodiments, the grains 60 of matrix material 52 may have a relatively smaller size (e.g., an average grain size of about six microns (6  $\mu$ m) or less) to impart increased hardness to the matrix material 52, while in other embodiments, the grains 60 of matrix material 52 may have a relatively larger size (e.g., an average grain size of greater than six microns (6  $\mu$ m)) to impart increased toughness to the matrix material 52. The size and shape of the grains 60 may be selectively tailored using heat treatments such as, for example, quenching and annealing, as known in the art. Furthermore, at least trace amounts of at least one of titanium and boron optionally may be included in the matrix material 52 to facilitate grain size refinement.

Referring again to FIG. 1, the bit body 12 may be secured to the metal shank 20 by way of, for example, a threaded connection 22 and a weld 24 that extends around the drill bit 10 on an exterior surface thereof along an interface between the bit body 12 and the metal shank 20. The metal shank 20 may be formed from steel, and may include a threaded pin 28 conforming to American Petroleum Institute (API) standards for attaching the drill bit 10 to a drill string (not shown).

As shown in FIG. 1, the bit body 12 may include wings or blades 30 that are separated from one another by junk slots 32. Internal fluid passageways 42 may extend between the face 18 of the bit body 12 and a longitudinal bore 40, which extends through the steel shank 20 and at least partially through the bit body 12. In some embodiments, nozzle inserts (not shown) may be provided at the face 18 of the bit body 12 within the internal fluid passageways 42.

The drill bit 10 may include a plurality of cutting structures on the face 18 thereof. By way of example and not limitation, a plurality of polycrystalline diamond compact (PDC) cutters 34 may be provided on each of the blades 30, as shown in FIG. 1. The PDC cutters 34 may be provided along the blades 30 within pockets 36 formed in the face 18 of the bit body 12, and may be supported from behind by buttresses 38, which may be integrally formed with the crown region 14 of the bit body 12.

The steel blank 16 shown in FIG. 1 may be generally cylindrically tubular. In additional embodiments, the steel blank 16 may have a fairly complex configuration and may include external protrusions corresponding to blades 30 or other features extending on the face 18 of the bit body 12.

The rotary drill bit 10 shown in FIG. 1 may be fabricated by separately forming the bit body 12 and the shank 20, and then attaching the shank 20 and the bit body 12 together. The bit body 12 may be formed by a variety of techniques, some of which are described in further detail below.

In some embodiments, the bit body 12 may be formed using so-called "suspension" or "dispersion" casting techniques. For example, a mold (not shown) may be provided that includes a mold cavity having a size and shape corresponding to the size and shape of the bit body 12. The mold may be formed from, for example, graphite or any other high-temperature refractory material, such as a ceramic. The mold cavity of the mold may be machined using a five-axis machine tool.

machine tool. Fine features may be added to the cavity of the mold using hand-held tools. Additional clay work also may be required to obtain the desired configuration of some features of the bit body 12. Where necessary, preform elements or displacements (which may comprise ceramic components, graphite components, or resin-coated sand compact components) may be positioned within the mold cavity and used to define the internal passageways 42, cutting element pockets 36, junk slots 32, and other external topographic features of the bit body 12.

After forming the mold, a suspension may be prepared that includes a plurality of silicon carbide particles 50 (FIG. 2) suspended within molten matrix material 52. Molten matrix material 52 having a composition as previously described herein then may be prepared by mixing stock material, particulate material, and/or powder material of each of the various elemental constituents in their respective weight percentages in a container and heating the mixture to a temperature sufficient to cause the mixture to melt, forming a molten matrix material 52 of desired composition. After forming the molten matrix material 52 of desired composition, silicon carbide particles 50 may be suspended and dispersed throughout the molten matrix material 52 to form the suspension. As previously mentioned, in some embodiments, the silicon carbide particles 50 may be coated with a material configured to enhance the wettability of the silicon carbide particles 50 to the molten matrix material 52 and/or to prevent any detrimental chemical reaction from occurring between the silicon carbide particles 50 and the molten matrix material 52. By way of example and not limitation, the silicon carbide particles 50 may comprise a coating of tin oxide (SnO<sub>2</sub>).

Optionally, a metal blank 16 (FIG. 1) may be at least partially positioned within the mold such that the suspension may be cast around the metal blank within the mold.

The suspension comprising the silicon carbide particles 50 and molten matrix material 52 may be poured into the mold cavity of the mold. As the molten matrix material (e.g., molten aluminum or aluminum-based alloy materials) may be susceptible to oxidation, the infiltration process may be carried out under vacuum. In additional embodiments, the molten matrix material may be substantially flooded with an inert gas or a reductant gas to prevent oxidation of the molten matrix material. In some embodiments, pressure may be applied to the suspension during casting to facilitate the casting process and to substantially prevent the formation of voids within the bit body 12 being formed.

After casting the suspension within the mold, the molten matrix material 52 may be allowed to cool and solidify, forming the solid matrix material 52 of the particle-matrix composite material 15 around the silicon carbide particles 50.

In some embodiments, the bit body 12 may be formed using so-called "infiltration" casting techniques. For example, a mold (not shown) may be provided that includes a mold cavity having a size and shape corresponding to the size and shape of the bit body 12. The mold may be formed from, for example, graphite or any other high-temperature refractory material, such as a ceramic. The mold cavity of the mold may be machined using a five-axis machine tool. Fine features may be added to the cavity of the mold using hand-held tools. Additional clay work also may be required to obtain the desired configuration of some features of the bit body 12. Where necessary, preform elements or displacements (which may comprise ceramic components, graphite components, or resin-coated sand compact components) may be positioned within the mold cavity and used to define the internal passageways 42, cutting element pockets 36, junk slots 32, and other external topographic features of the bit body 12.

After forming the mold, a plurality of silicon carbide particles **50** (FIG. 2) may be provided within the mold cavity to form a body having a shape that corresponds to at least the crown region **14** of the bit body **12**. Optionally, a metal blank **16** (FIG. 1) may be at least partially embedded within the silicon carbide particles **50** such that at least one surface of the blank **16** is exposed to allow subsequent machining of the surface of the metal blank **16** (if necessary) and subsequent attachment to the shank **20**.

Molten matrix material **52** having a composition as previously described herein then may be prepared by mixing stock material, particulate material, and/or powder material of each of the various elemental constituents in their respective weight percentages, heating the mixture to a temperature sufficient to cause the mixture to melt, thereby forming a molten matrix material **52** of desired composition. The molten matrix material **52** then may be allowed or caused to infiltrate the spaces between the silicon carbide particles **50** within the mold cavity. Optionally, pressure may be applied to the molten matrix material **52** to facilitate the infiltration process as necessary or desired. As the molten materials (e.g., molten aluminum or aluminum-based alloy materials) may be susceptible to oxidation, the infiltration process may be carried out under vacuum. In additional embodiments, the molten materials may be substantially flooded with an inert gas or a reductant gas to prevent oxidation of the molten materials. In some embodiments, pressure may be applied to the molten matrix material **52** and silicon carbide particles **50** to facilitate the infiltration process and to substantially prevent the formation of voids within the bit body **12** being formed.

After the silicon carbide particles **50** have been infiltrated with the molten matrix material **52**, the molten matrix material **52** may be allowed to cool and solidify, forming the solid matrix material **52** of the particle-matrix composite material **15**.

In additional embodiments, reactive infiltration casting techniques may be used to form the bit body **12**. By way of example and not limitation, the mass to be infiltrated may comprise carbon, and molten silicon may be added to the molten matrix material **50**. The molten silicon may react with the carbon to form silicon carbide as the molten mixture infiltrates the carbon material. In this manner, a reaction may be used to form silicon carbide particles **52** in situ during the infiltration casting process.

In some embodiments, the bit body **12** may be formed using so-called particle compaction and sintering techniques such as, for example, those disclosed in pending application Ser. No. 11/271,153, filed Nov. 10, 2005, and pending application Ser. No. 11/272,439, filed Nov. 10, 2005. Briefly, a powder mixture may be pressed to form a green bit body or billet, which then may be sintered one or more times to form a bit body **12** having a desired final density.

The powder mixture may include a plurality of silicon carbide particles **52** and a plurality of particles comprising a matrix material **50**, as previously described herein. Optionally, the powder mixture may further include additives commonly used when pressing powder mixtures such as, for example, binders for providing lubrication during pressing and for providing structural strength to the pressed powder component, plasticizers for making the binder more pliable, and lubricants or compaction aids for reducing inter-particle friction. Furthermore, the powder mixture may be milled, which may result in the silicon carbide particles **52** being at least partially coated with matrix material **50**.

The powder mixture may be pressed (e.g., axially within a mold or die, or substantially isostatically within a mold or

container) to form a green bit body. The green bit body may be machined or otherwise shaped to form features such as blades, fluid courses, internal longitudinal bores, cutting element pockets, etc., prior to sintering. In some embodiments, the green bit body (with or without machining) may be partially sintered to form a brown bit body, and the brown bit body may be machined or otherwise shaped to form one or more such features prior to sintering the brown bit body to a desired final density.

10 The sintering processes may include conventional sintering in a vacuum furnace, sintering in a vacuum furnace followed by a conventional hot isostatic pressing process, and sintering immediately followed by isostatic pressing at temperatures near the sintering temperature (often referred to as sinter-HIP). Furthermore, the sintering processes may include subliquidus phase sintering. In other words, the sintering processes may be conducted at temperatures proximate to but below the liquidus line of the phase diagram for the matrix material. For example, the sintering processes described herein may be conducted using a number of different methods known to one of ordinary skill in the art, such as the Rapid Omnidirectional Compaction (ROC) process, the CERACONTM process, hot isostatic pressing (HIP), or adaptations of such processes.

15 20 25 When the bit body **12** is formed by particle compaction and sintering techniques, the bit body **12** may not include a metal blank **16** and may be secured to the shank **20** by, for example, one or more of brazing, welding, and mechanically interlocking.

30 As previously mentioned, in some embodiments, the silicon carbide particles **50** may comprise an in situ toughened ABC—SiC material. In such embodiments, the bit body **12** may be formed by various methods, including those described below.

35 40 45 In some embodiments of methods of forming a bit body **12** of the present invention, particles of ABC—SiC may be consolidated to form relatively larger structures or compacts by, for example, hot pressing particles of ABC—SiC at elevated temperatures (e.g., between about 1,650° C. and about 1,950° C.) and pressures (e.g., about fifty megapascals (50 MPa)) for a period of time (e.g., about one hour) in an inert gas (e.g., argon).

50 After consolidation of the ABC—SiC particles to form relatively larger compacts, the compacts may be annealed to 45 tailor the size and shape of the SiC grains in a manner that enhances the fracture toughness of the ABC—SiC material (e.g., to toughen the ABC—SiC material in situ). By way of example, the relatively larger compacts may be annealed at elevated temperatures (e.g., about 1,000° C. or more) for a time period of about one hour or more) in an inert gas.

55 The consolidated and annealed compacts then may be crushed or otherwise broken up (e.g., in a ball mill or an attritor mill) to form relatively smaller silicon carbide particles **52** comprising the in situ toughened ABC—SiC material. Optionally the relatively smaller silicon carbide particles **52** comprising the in situ toughened ABC—SiC material may be screened to separate the particles into certain particle size ranges, and only selected particle size ranges may be used in forming the bit body **12**. The silicon carbide particles **52** comprising the in situ toughened ABC—SiC material then 60 may be used to form the bit body **12** by, for example, using any of the suspension casting, infiltration casting, or particle compaction and sintering methods previously described herein.

65 In additional embodiments of methods of forming a bit body **12** of the present invention, particles of ABC—SiC may be consolidated to form relatively larger compacts as previ-

## 11

ously described. Prior to annealing (and in situ toughening of the ABC—SiC), however, the relatively larger compacts may be crushed or broken up to form relatively smaller silicon carbide particles **52** comprising the ABC—SiC material. The silicon carbide particles **52** comprising the ABC—SiC material then may be used to form the bit body **12** by, for example, using any of the suspension casting, infiltration casting, or particle compaction and sintering methods previously described herein. A matrix material **50** may be used that has a sufficiently high melting point (e.g., greater than about 1,250° C.) to allow annealing and in situ toughening of the ABC—SiC material after forming the hit body **12** without causing incipient melting of the matrix material **50** or undue dissolution between the matrix material **50** and the silicon carbide particles **52**. Such matrix materials **50** may include, for example, cobalt, cobalt-based alloys, nickel, nickel-based alloys, or a combination of such materials. In this manner, the ABC—SiC material may be in situ toughened after forming the bit body **12**.

In further embodiments of methods of forming a bit body **12** of the present invention, particles of ABC—SiC may be consolidated to form a first set of relatively larger compacts as previously described. Prior to annealing (and in situ toughening of the ABC—SiC), however, the relatively larger compacts may be crushed or broken up to form relatively smaller silicon carbide particles comprising the ABC—SiC material. A second set of relatively larger compacts may be formed by infiltrating (or otherwise consolidating) the silicon carbide particles **52** comprising the ABC—SiC material with a first material that has a sufficiently high melting point (e.g., greater than about 1,250° C.) to allow annealing and in situ toughening of the ABC—SiC material after infiltrating with the first material. The second set of compacts then may be annealed and in situ toughened, as previously described, after which the second set of compacts may be crushed or otherwise broken up to form the relatively smaller silicon carbide particles **52** comprising in situ toughened ABC—SiC material. The silicon carbide particles **52** comprising the in situ toughened ABC—SiC material then may be used to form the bit body **12** by, for example, using any of the suspension casting, infiltration casting, or particle compaction and sintering methods previously described herein. A matrix material **50** may be used having a melting point such that the bit body **12** may be formed without causing incipient melting of the first material (which is used to infiltrate the ABC—SiC particles prior to in situ toughening), or undue dissolution between the matrix material **50** and the first material or the silicon carbide particles **52**.

After or during formation of the bit body **12**, the bit body **12** optionally may be subjected to one or more thermal treatments (different than in situ toughening, as previously described) to selectively tailor one or more physical properties of at least one of the matrix material **52** and the silicon carbide particles **50**.

For example, the matrix material **52** may be subjected to a precipitation hardening process to form a discontinuous phase **56** comprising precipitates, as previously described in relation to FIG. 4. For example, the matrix material **52** may comprise between about 95% and about 96.5% by weight aluminum and between about 3.5% and about 5% by weight copper, as previously described. In fabricating the bit body **12** in an infiltration casting type process, as described above, the matrix material **52** may be heated to a temperature of greater than about 548° C. (a eutectic temperature for the particular alloy) for a sufficient time to allow the composition of the molten matrix material **52** to become substantially homogeneous. The substantially homogenous molten matrix material

## 12

**52** may be poured into a mold cavity and allowed to infiltrate the spaces between silicon carbide particles **50** within the mold cavity. After substantially complete infiltration of the silicon carbide particles **50**, the temperature of the molten matrix material **52** may be cooled relatively rapidly (i.e., quenched) to a temperature of less than about 100° C. to cause the matrix material **52** to solidify without formation of a significant amount of discontinuous precipitate phases. The temperature of the matrix material **52** then may be heated to a temperature of between about 100° C. and about 548° C. for a sufficient amount of time to allow the formation of a selected amount of discontinuous precipitate phase (e.g., metastable transition precipitation phases, and/or equilibrium precipitation phases). In additional embodiments, the composition of the matrix material **52** may be selected to allow a pre-selected amount of precipitation hardening within the matrix material **52** over time and under ambient temperatures and/or temperatures attained while drilling with the drill bit **10**, thereby eliminating the need for a heat treatment at elevated temperatures.

Tungsten carbide materials have been used for many years to form bodies of earth-boring tools. Silicon carbide generally exhibits higher hardness than tungsten carbide materials. Silicon carbide materials also may exhibit superior wear resistance and erosion resistance relative to tungsten carbide materials. Therefore, embodiments of the present invention may provide earth-boring tools that exhibit relatively higher hardness, improved wear resistance, and/or improved erosion resistance relative to conventional tools comprising tungsten carbide composite materials. Furthermore, by employing toughened silicon carbide materials, as disclosed herein, earth-boring tools may be provided that comprise silicon carbide composite materials that exhibit increased fracture toughness.

While the present invention is described herein in relation to embodiments of concentric earth-boring rotary drill bits that include fixed cutters and to embodiments of methods for forming such drill bits, the present invention also encompasses other types of earth-boring tools such as, for example, core bits, eccentric bits, bicenter bits, reamers, mills, and roller cone bits, as well as methods for forming such tools. Thus, as employed herein, the term “bit body” includes and encompasses bodies of all of the foregoing structures, as well as components and subcomponents of such structures.

While the present invention has been described herein with respect to certain preferred embodiments, those of ordinary skill in the art will recognize and appreciate that it is not so limited. Rather, many additions, deletions and modifications to the preferred embodiments may be made without departing from the scope of the invention as hereinafter claimed. In addition, features from one embodiment may be combined with features of another embodiment while still being encompassed within the scope of the invention as contemplated by the inventors. Further the invention has utility in drill bits and core bits having different and various bit profiles as well as cutter types.

What is claimed is:

1. A method of forming an earth-boring tool, the method comprising:

providing a silicon carbide material comprising between about one percent by weight (1.0 wt %) and about five percent by weight (5.0 wt %) aluminum, less than about one percent by weight (1.0 wt %) boron, and between about one percent by weight (1.0 wt %) and about four percent by weight (4.0 wt %) carbon; consolidating the silicon carbide material to form at least one compact;

## 13

breaking apart the at least one compact to form a plurality of silicon carbide particles; providing a bit body comprising: providing a green powder component comprising: at least some of the plurality of silicon carbide particles; and a plurality of particles each comprising aluminum or an aluminum-based alloy material; and at least partially sintering the green powder component; providing a shank that is configured for attachment to a drill string; and attaching the shank to the bit body.

2. The method of claim 1, wherein providing a green powder component comprises:

providing a powder mixture comprising: the at least some of the plurality of silicon carbide particles; the plurality of silicon carbide particles each comprising an aluminum or aluminum-based alloy material; and a binder material; and pressing the powder mixture.

3. The method of claim 1, wherein at least partially sintering the green powder component comprises:

partially sintering the green powder component to form a brown bit body; machining at least one feature in a surface of the brown bit body; and sintering the brown bit body to a desired final density.

4. A method of forming an earth-boring tool, the method comprising:

providing a silicon carbide material comprising between about one percent by weight (1.0 wt %) and about five percent by weight (5.0 wt %) aluminum, less than about one percent by weight (1.0 wt %) boron, and between about one percent by weight (1.0 wt %) and about four percent by weight (4.0 wt %) carbon;

consolidating the silicon carbide material to form at least one compact;

breaking apart the at least one compact to form a plurality of silicon carbide particles;

providing the plurality of silicon carbide particles in an aluminum or aluminum alloy matrix material to form a body; and

shaping the body to form at least a portion of an earth-boring tool for drilling subterranean formations.

5. The method of claim 4, wherein the providing the plurality of silicon carbide particles in an aluminum or aluminum alloy matrix material to form a body, and the shaping the body to form at least a portion of an earth-boring tool for drilling subterranean formations, further comprise infiltrating the plurality of silicon carbide particles in a cavity of a mold having a shape corresponding to the at least a portion of the body of an earth-boring tool for drilling subterranean formations with the matrix material.

6. The method of claim 5, further comprising toughening the silicon carbide particles prior to infiltrating the plurality of silicon carbide particles with the matrix material.

7. The method of claim 6, wherein toughening the silicon carbide particles comprises annealing at least one compact

## 14

comprising silicon carbide material to alter at least one of the size and shape of silicon carbide grains within the at least one compact.

8. The method of claim 5, further comprising toughening the silicon carbide particles after infiltrating the plurality of silicon carbide particles with the matrix material.

9. The method of claim 4, wherein the providing the plurality of silicon carbide particles in an aluminum or aluminum alloy matrix material to form a body, and the shaping the body to form at least a portion of an earth-boring tool for drilling subterranean formations, further comprise:

pressing a powder mixture comprising the plurality of silicon carbide particles and a plurality of particles comprising the matrix material to form a green powder component; and

at least partially sintering the green powder component.

10. The method of claim 9, further comprising toughening the silicon carbide particles prior to pressing the powder mixture.

11. The method of claim 4, further comprising causing the matrix material to comprise at least 75% by weight aluminum and at least trace amounts of at least one of boron, carbon, copper, iron, lithium, magnesium, manganese, nickel, scandium, silicon, tin, zirconium, and zinc.

12. A method of forming at least a portion of a body of an earth-boring tool, the method comprising:

providing a silicon carbide material comprising between about one percent by weight (1.0 wt %) and about five percent by weight (5.0 wt %) aluminum, less than about one percent by weight (1.0 wt %) boron, and between about one percent by weight (1.0 wt %) and about four percent by weight (4.0 wt %) carbon;

consolidating the silicon carbide material to form at least one compact;

breaking apart the at least one compact to form a plurality of silicon carbide particles; and

forming at least a portion of a body of an earth-boring tool to comprise a composite material comprising the plurality of silicon carbide particles and an aluminum or aluminum alloy particles and a matrix material.

13. The method of claim 12, further comprising annealing the at least one compact to increase a fracture toughness exhibited by the silicon carbide material.

14. The method of claim 12, further comprising annealing the silicon carbide material to increase a fracture toughness exhibited by the silicon carbide material.

15. The method of claim 1, further comprising annealing the at least one compact comprising the silicon carbide material to alter at least one of the size and shape of silicon carbide grains within the at least one compact.

16. The method of claim 15, wherein annealing the at least one compact comprises toughening the silicon carbide material.

17. The method of claim 10, wherein toughening the silicon carbide particles comprises annealing the at least one compact comprising the silicon carbide material to alter at least one of the size and shape of silicon carbide grains within the at least one compact.

\* \* \* \* \*

UNITED STATES PATENT AND TRADEMARK OFFICE  
**CERTIFICATE OF CORRECTION**

PATENT NO. : 7,807,099 B2  
APPLICATION NO. : 11/965018  
DATED : October 5, 2010  
INVENTOR(S) : Heeman Choe et al.

Page 1 of 2

It is certified that error appears in the above-identified patent and that said Letters Patent is hereby corrected as shown below:

**On the title page:**

In ITEM (54) **TITLE** change “METHOD” to --METHODS--

In ITEM (56) **References Cited**

U.S. PATENT DOCUMENTS

Page 1, 1<sup>st</sup> Column, 10<sup>th</sup> entry, line 54 change “6,503,572 B1 1/2003 Aghajanian et al.”  
to --6,503,572 B1 1/2003 Waggoner et al.--  
Page 1, 1<sup>st</sup> Column, 11<sup>th</sup> entry, line 55 change “6,862,970 B2 3/2005 Waggoner et al.”  
to --6,862,970 B2 3/2005 Aghajanian et al.--

In ITEM (56) **References Cited**

OTHER PUBLICATIONS

1<sup>st</sup> Page, 2<sup>nd</sup> Column, 2<sup>nd</sup> line of 6<sup>th</sup> entry, line 19 change “Si3N4/6061” to --Si<sub>3</sub>N<sub>4</sub>/6061--  
1<sup>st</sup> Page, 2<sup>nd</sup> Column, 2<sup>nd</sup> line of 9<sup>th</sup> entry, line 29 change “mater,” to --mater.--  
1<sup>st</sup> Page, 2<sup>nd</sup> Column, 2<sup>nd</sup> line of 10<sup>th</sup> entry, line 32 change “10wt.% Sic” to --10 wt.% SiC--  
1<sup>st</sup> Page, 2<sup>nd</sup> Column, 2<sup>nd</sup> line of 11<sup>th</sup> entry, line 35 change “Sicp Coated by SnO<sub>2</sub>,”  
to --SiCp Coated by SnO<sub>2</sub>,--  
1<sup>st</sup> Page, 2<sup>nd</sup> Column, 3<sup>rd</sup> line of 12<sup>th</sup> entry, line 39 change “mater,” to --mater.--

**In the specification:**

COLUMN 1, LINE 1, change “METHOD” to --METHODS--  
COLUMN 3, LINE 60, change “bow” to --how--  
COLUMN 4, LINE 44, change “gains” to --grains--  
COLUMN 11, LINE 12, change “hit body” to --bit body--

Signed and Sealed this  
Nineteenth Day of June, 2012



David J. Kappos  
Director of the United States Patent and Trademark Office

**CERTIFICATE OF CORRECTION (continued)**  
**U.S. Pat. No. 7,807,099 B2**

Page 2 of 2

**In the claims:**

CLAIM 5, COLUMN 13, LINE 50,

change "comprise" to --comprises--

CLAIM 9, COLUMN 14, LINE 11,

change "comprise:" to --comprises:--

CLAIM 12, COLUMN 14, LINE 40,

change "alloy particles and a matrix" to --alloy a

matrix--